

April 14, 1953

J. F. VOGT ET AL

2,635,075

PLATING PROCESS

Filed Feb. 28, 1948



INVENTORS  
JOHN F. VOGT &  
RUSSEL J. HERBERT  
BY *Bair & Freeman*  
ATTYS.

## UNITED STATES PATENT OFFICE

2,635,075

## PLATING PROCESS

John F. Vogt and Russell J. Herbert, St. Louis,  
Mo., assignors to Knapp-Monarch Company,  
St. Louis, Mo., a corporation of Delaware

Application February 28, 1948, Serial No. 12,032

3 Claims. (Cl. 204—49)

1

This invention relates to a nickel plating process wherein an object after being plated in accordance with our process requires a minimum of polishing and practically no buffing at all providing a Watts nickel bath containing coumarin (as disclosed in the Harshaw British Patent No. 622,761) is used.

One object of the invention is to provide a plating process which involves certain steps that permit the final plating of an object with a bright nickel solution that adheres in a superior manner to the object and does not subsequently blister as with ordinary processes, the use of our process requiring less polishing and buffing than ordinary bright nickel plating providing a Watts nickel plating bath containing coumarin (as disclosed in the Harshaw British Patent No. 622,761) is used preceding bright nickel plating carried out according to the Harshaw Patents Nos. 2,029,386, 2,029,387, 2,125,229, 2,198,267, 2,198,268, 2,290,342, 2,238,661 or 2,326,999.

Another object is to provide a process involving the steps of nickel plating in a Watts nickel bath containing coumarin (as disclosed in the Harshaw British Patent No. 622,761) and bright nickel plating with an intermediate step wherein the work is subjected to a few seconds of reverse current flow and then to a somewhat longer period of current flow in the normal (from anode to work) direction in a solution of sodium cyanide and sodium carbonate, this particular step of the process resulting in elimination of blistering and reduction of the necessity for polishing and buffing, which are required in connection with nickel plating in a Watts bath containing coumarin but less so with bright nickel plating according to the above identified Harshaw United States patents, the step of subjecting the work to the sodium cyanide and sodium carbonate solution being the means to eliminate subsequent blistering and minimizing the polishing and buffing operations.

More specifically, it is our object to provide an intermediate step between nickel plating in a Watts bath containing coumarin and bright nickel plating according to the above identified Harshaw United States patents which deplates the first layer of nickel plating for about two to five seconds and then replates for approximately twenty seconds in a sodium cyanide-sodium carbonate solution wherein the proportions are approximately 5 to 1 to secure best results.

With these and other objects in view, our invention consists in the specific steps of the process hereinafter outlined whereby the ob-

jects are attained as will be evident from the following description, pointed out in our claims and illustrated in the accompanying drawings, wherein:

5 Figure 1 is a diagrammatic view of the first step of our process consisting of nickel plating.

Figure 2 is a similar diagrammatic view of the second step of our process consisting of deplating.

Figure 3 is a similar diagrammatic view of the third step of our process wherein the work is replated, and

Figure 4 is a similar diagrammatic view of the final step of the process which consists of bright nickel plating.

The process of bright nickel plating heretofore has involved substantially two steps. The first step is to plate in a nickel solution and the second step is to plate in a bright nickel solution. 10 Various solutions have been discovered and used for general commercial work such as the plating of electrical appliances.

To improve upon the nickel plating process as just described however we have devised an intermediate step between the nickel plating and the bright nickel plating steps thereof and our particular process will now be described after a brief description as to how the first nickel plating step is accomplished.

15 In Figure 1 we illustrate a plating tank 10 having therein a plating solution 12 which is an ordinary nickel plating solution or a Watts bath containing coumarin as disclosed in Harshaw British Patent No. 622,761. An anode is illustrated at 14 and the article to be plated (work) is illustrated at 16. A wire 18 is connected with the anode to supply current from the positive terminal of a suitable current supply and the negative wire thereof indicated at 20 is connected with the work 16. The usual nickel plating is then done 20 by energizing the circuit so that current flows and nickel is deposited from the anode 14 and plated on the work 16, the direction of nickel flow being indicated by the arrow 22.

25 The next step in our plating process is to place the work 16 in a tank 24 containing a solution 26 of six to sixteen ounces of sodium cyanide (10 ounces being preferable), two to ten ounces of sodium carbonate (2 ounces being preferable) in one gallon of water. Or, according to the metric system: 45 to 120 grams of sodium cyanide per liter of water, 75 grams being preferred, together with from 15 to 75 grams of sodium carbonate per liter of water, 15 grams being preferred. Four 30 to ten volts (6 volts preferred) current is then

passed in a reverse direction through the solution 26—that is the positive wire 18 is connected with work and the negative wire 20 is connected with the anode. The direction of flow is then from the work toward the anode as indicated by the arrow 28. The duration of flow of current is preferably from two to five seconds.

The next step illustrated in Figure 3 is to reverse the direction of the current by connecting the positive wire 18 to the anode 14 and the negative wire 20 to the work 16, the anode and work still being suspended in the solution 26 already referred to in connection with Figure 2. The direction of current flow will now be in the normal or plating direction as indicated by the arrow 30. We have found that approximately twenty seconds is satisfactory for the duration of current flow in the replating direction.

After the third step in the process the work is rinsed in clear water and then suspended in another tank 32 having a solution 34 therein which is a bright nickel solution such as any of the solutions disclosed in the above noted Harshaw United States patents. The direction of current flow is again in the normal plating direction as indicated by the arrow 36, the wires 18 and 20 being suitably connected to the anode and work for flow of bright nickel in the proper direction through the solution 34—that is from the anode to the work.

The intermediate steps illustrated in Figures 2 and 3 eliminate the blistering which readily occurs when articles are plated without such intermediate step. We have indicated certain proportions for the solution 26 and certain voltages and timing for the current flow but this can vary to some extent and still secure satisfactory results. We have however indicated what we have found to be the best proportions, voltages and timing.

The resulting product from ordinary nickel plating and bright nickel plating is only fair. Our process involving the intermediate steps illustrated in Figures 2 and 3 improves upon the former processes, as the resulting product does not blister and requires but a minimum of polishing and practically no buffing. A longer lasting surface is thereby provided for electrical appliances and the like when our method is used and the finished product is attained with much less manual work at the factory in connection with handling of appliances involving the necessity of polishing and buffing them to bring out the luster of the finish. With our process this work and the time consumed by it is reduced to a minimum so that many more articles per day can be produced by the same number of workmen.

Some changes may be practiced in the steps of our process without departing from the real spirit and purpose of our invention. Accordingly, it is our intention to cover by our claims such deviations from the steps specifically enumerated as may be reasonably included within their scope.

We claim as our invention:

1. A method of preparing an article for electro-deposition thereon of a coating of bright nickel, said method comprising making said article the cathode in a first bath, thereafter making said article the anode for two to five seconds in a second bath, said first bath being a Watts nickel bath containing coumarin and said second bath consisting essentially of from 45 to 120 grams of sodium cyanide and from 15 to 75 grams of sodium carbonate per liter of water, the voltage in said second bath being from 4 to 10, and thereafter reversing the current in said second bath to make said article the cathode at said voltage for about twenty seconds.

2. A method of preparing an article for electro-deposition thereon of a coating of bright nickel, said method comprising making said article the cathode in a first bath, thereafter making said article the anode for two to five seconds in a second bath, said first bath being a Watts nickel bath containing coumarin and said second bath consisting essentially of from 45 to 120 grams of sodium cyanide and from 15 to 75 grams of sodium carbonate per liter of water, the voltage in said second bath being from 4 to 10, thereafter reversing the current in said second bath to make said article the cathode in said voltage for about twenty seconds and thereafter rinsing said article with water.

3. A method of preparing an article for electro-deposition thereon of a coating of bright nickel, said method comprising making said article the cathode in a first bath, thereafter making said article the anode for two to five seconds in a second bath, said first bath being a Watts nickel bath containing coumarin and said second bath consisting essentially of about 75 grams of sodium cyanide and about 15 grams of sodium carbonate per liter of water, the voltage in said second bath being about 6, thereafter reversing the current in said second bath to make said article the cathode at said voltage for about twenty seconds, and thereafter rinsing said article with water.

JOHN F. VOGT.  
RUSSELL J. HERBERT.

References Cited in the file of this patent

UNITED STATES PATENTS

| Number    | Name             | Date           |
|-----------|------------------|----------------|
| 93,157    | Adams            | Aug. 3, 1869   |
| 1,534,709 | Holt             | Apr. 21, 1925  |
| 1,574,055 | Pedersen         | Feb. 23, 1926  |
| 1,918,605 | Jones            | July 18, 1933  |
| 2,384,660 | Ward             | Sept. 11, 1945 |
| 2,451,341 | Jernstedt        | Oct. 12, 1948  |
| 2,470,775 | Jernstedt et al. | May 24, 1949   |

OTHER REFERENCES

Metal Finishing, pages 68-72, 1947.